

# UNITED STATES PATENT OFFICE.

HEINRICH SCHOWALTER, OF LADENBURG, GERMANY.

## OIL-DRESSING FOR LEATHER.

No. 821,260.

Specification of Letters Patent.

Patented May 22, 1906.

Application filed October 25, 1905. Serial No. 284,314.

*To all whom it may concern:*

Be it known that I, HEINRICH SCHOWALTER, a citizen of the Empire of Germany, residing at Ladenburg, Baden, Germany, have invented certain new and useful Improvements in Oil-Dressings for Leather, of which the following is a specification.

A standard leather-preserving oil which can act at the same time as an impregnating material must fulfil the following requirements: It must, first, be able to penetrate easily into the leather without leaving a layer of fat behind or transpiring; secondly, it must hold well in the leather and must not be capable of being soaked out by air, water, steam, &c.; thirdly, it must make the leather permanently soft, flexible, and water-tight.

According to this invention such a leather-preserving oil is composed of a good train-oil to which has been added anilin-oil and a solution of india-rubber in turpentine. Pure train-oil is too thick to penetrate rapidly into the leather. Moreover, it leaves a layer of grease and transpires, and also it does not remain in the leather, but can be easily driven out by water because it is lighter than the latter. By the addition of anilin-oil and a solution of india-rubber in turpentine it is rendered more limpid, penetrates immediately on application into the leather, and remains firmly therein. Air, water, or steam have no influence upon the leather treated with this admixture of materials. The leather consequently remains permanently soft, flexible, and waterproof.

Experiments which have been made have proved that when a three-per-cent. solution of india-rubber in turpentine in a quantity of, say, ten liters was added to ninety liters of a pure train-oil the mixture could still be driven out of the leather by water, but that it remained permanently therein if only one and one-half per cent. of anilin-oil was intermixed. In these experiments three bags of sheep-leather were made use of, because this leather is very porous. The first bag was treated inside on the flesh side of the leather with train-oil, the second bag with train-oil to which a solution of rubber in turpentine of three per cent. was added, and the third bag was treated with train-oil to which a suitable quantity of a three-per-cent. solution of rubber in turpentine and one and one-half per cent. of anilin-oil was added. Each bag was filled with water and suspended on the wall. After a short time the water began to force

out the oil from the leather of the first bag. The leather became very oily on the outside, and this oil collected in great drops at the under part of the bag, which drops at first slowly, and subsequently more quickly, fell to the ground until all the oil was driven out of the leather and the water itself began to drop. With the second bag it required considerably longer time before the oil began to drop and the water followed it out of the bag, but finally this bag also dropped until it was empty. Only the third bag retained the water for weeks. No oil was visible upon the outside of the sheep-leather bag and the leather remained soft and elastic. This result was very surprising because the anilin-oil was added primarily to counteract the acids present rather than specially to render the leather water-tight. The experiments, however, have been repeated several times for the purpose of ascertaining in what manner the water-tight effect is produced by the addition of anilin-oil to train-oil mixed with three-per-cent.-rubber solution in turpentine, and it has been discovered that by the addition of the anilin this combines with the turpentine and the rubber is separated. It is therefore possible that a similar action takes place in the leather, so that the water-tightness is really effected by the rubber alone.

According to the quality and thickness of the leather treated the quantity of the rubber solution has to be proportionately increased or decreased.

Having now particularly described and ascertained the nature of my said invention and in what manner the same is to be performed, I declare that what I claim is—

1. An improved preparation for the preservation and waterproofing of leather, consisting of train-oil mixed with a suitable quantity of a three-per-cent. solution of india-rubber in turpentine and one and one-half per cent. of anilin-oil.

2. A preparation for the preservation and waterproofing of leather, consisting of a train-oil mixed with anilin-oil and a solution of india-rubber in turpentine.

In testimony that I claim the foregoing as my invention I have signed my name in presence of two subscribing witnesses.

HEINRICH SCHOWALTER.

Witnesses:

AUG. NEIMINTUNG,  
Jos. H. LEUTE.